

## UNITED STATES PATENT OFFICE.

EMIL HENE, OF STASSFURT, GERMANY.

## PROCESS OF PRODUCING DECOLORIZING CARBON.

No Drawing.

Application filed July 18, 1924. Serial No. 726,830.

*To all whom it may concern:*

Be it known that I, EMIL HENE, citizen of the German Republic, residing at 5 Sulze-strasse, Stassfurt, Germany, have invented new and useful Improvements in a Process of Producing Decolorizing Carbon, of which the following is a specification.

This invention relates to an improved process of producing the so called active or decolorizing carbon, its object being to produce highly efficient decolorizing carbon having a strong decolorizing power on the usual liquids to be decolorized by relatively simple and inexpensive operations and from cheap ingredients.

Regarding the present state of the decolorizing carbon producing art of which I am aware, I know, that it has already been proposed to produce decolorizing carbon from mineral coal such as brown coal or other bituminous or carbonaceous matter by heating the same together with reducible substances, for example sulfates, at a suitable temperature. Of importance for any process of transforming carbonaceous matter into decolorizing carbon is the thorough-going action upon the carbon substance treated since otherwise the surface increase and roughening which is responsible for the decolorizing power cannot be obtained throughout the material. In order to secure this thorough-going effect it has further already been proposed (U. S. Patent 1,383,755 to Punnett and Whitaker), to start from vegetable substances to impregnate the same, after due comminution with a suitable sulfate solution, to char the substance thus impregnated at a relatively low temperature and to thereupon subject it to a second heat treatment at a considerably increased temperature after separation of the reduction substance from the charred carbonizable material. It has further been proposed to impregnate already existing mineral coal or carbon with the reduction sulfate by a consecutive impregnation with sulfate component solutions, thus depositing the sulfate within the very pores or interstices of the starting material (German Patent 248571 to Lotz). Finally it has already been proposed to mechanically mix the coal

or carbon with an alkaline earth sulfate and to subject the mixture to one heating operation at a relatively high temperature, whereupon the reduction substance is separated from the finished decolorizing carbon by a suitable cleansing operation and the carbon subjected, if necessary, to a short repeated heating (German Patent 310622 to Chemische Werke Carbon).

Contrary to all of these known processes my present invention is substantially based upon the discovery, that also alkali-metal-sulfur-compounds adapted to be reduced to a sulfide by coal or carbon at a suitable temperature can also be used with particular advantage for the production of an excellent decolorizing carbon by mixing them in a dissolved or undissolved condition with the mineral coal or carbon and heating the mixture at a temperature of more than 600° C. As such alkali-metal sulfur-compounds the sulfates and bisulfates of the alkali metals or the component mixtures of these alkali compounds may with particular advantage be used.

As a matter of fact the whole pertinent literature which I know states a process of mixing an alkali metal sulfate with mineral coal or carbon and of heating the mixture for the purpose of transforming the coal or carbon into active or decolorizing carbon as being impracticable. In contra-distinction to all of these statements I have discovered that also the alkali-metal-sulfur-compounds can be successfully used, provided that the heating operation is carried out for a sufficiently long period of time and at a temperature of at least 600° C. Since alkali metal sulfate and alkali metal bisulfate may sometimes, particularly upon use of coarse or large-grained coal or carbon not enter deeply enough into and clog the pores, one has been dissuaded entirely from the use of the alkali-metal-sulfur-compounds in mechanical mixture with the carbonaceous starting material. My experiments and practical factory work have however shown that just with the alkali-metal-sulfur-compounds an excellent decolorizing carbon can be obtained, particularly if the coal or carbon is comminuted before the heating oper-

ation into relatively small grains warranting the complete penetration with the sulfate or bisulfate to be reduced. If it is preferred not to comminute the carbonaceous matter 5 before the heating operation the process may also be carried out by first mixing the coal with a relatively limited quantity of the sulfate or bisulfate or of the component mixtures thereof, whereupon the reduction substance is separated after heating and the 10 whole procedure repeated until the desired thorough-going effect is secured, it being of course understood that such repeated treatment may also efficiently be used with matter 15 having before been comminuted into relatively small grains.

My process may be carried out with practically any mineral coal or carbon such as brown coal, bituminous coal, coke obtained 20 by a distillation of coal or brown coal and the like. Regarding the proportions of the mixture the same can be so chosen that the reacting mixture obtained becomes liquid or remains in a solid condition, so that the process 25 can be carried out with practically any type of furnace.

The use of the alkali metal sulfates or bisulfates or of their component mixtures as the substance to be reduced by the coal or 30 carbon so as to change the texture thereof is of manifest practical advantage as these compounds are by the formation of the decolorizing carbon transferred into the valuable and soluble alkali metal sulfides, where- 35 as upon the use of the alkaline earth sulfates the insoluble and valueless alkaline earth sulfides are produced which must be separated from the carbon by a cleansing operation, unlike the alkali metal sulfides which 40 can be readily dissolved out with water. Regarding the proposal to mix mineral coal with an alkaline earth sulfate and to heat the same at a high temperature it would even be of advantage to use the alkaline 45 earth bisulfates on account of their greater oxygen contents compared with the alkaline earth sulfate and of their accordingly more vigorous effect upon the carbon.

In carrying out my improved process 100 50 kg. of potassium sulfate were mixed with 80 kg. of charred brown coal and heated at 650-700° C. during ½-1 hour with the exclusion of oxygen or other oxidizing substance. After the heating the material was drawn 55 into a rather tightly closing receptacle, cooled down and treated with water, thereby forming a solution of sulfide which could be subjected to further separate treatment, whereas the finished active coal was left and 60 could be further purified according to its particular destination. In lieu of 100 kg. of potassium sulfate one may also use 130 kg. of barium sulfate. One may also replace the potassium sulfate for example by an 65 equivalent quantity of potassium chloride

and sulfuric acid or an equivalent quantity of potassium bisulfate or of its constituting components.

What I claim as my invention is:-

1. The process of producing decolorizing 70 carbon, comprising, mixing porous mineral coal with an alkali metal sulfur compound reducible to an alkali metal sulfide upon being heated with carbonaceous matter, heating the mixture at a temperature of at 75 least 600° C. and subsequently dissolving out the alkali metal compounds from the carbon.

2. The process of producing decolorizing 80 carbon, comprising, mechanically mixing porous mineral coal with an undissolved 85 alkali metal sulfur compound reducible to an alkali metal sulfide upon being heated with carbonaceous matter, heating the mixture at a temperature of at least 600° C., and dissolving out the alkali metal compounds from the carbon.

3. The process of producing decolorizing 90 carbon, comprising, mixing porous mineral coal with an alkali metal sulfate, heating the mixture at a temperature of at least 600° C., and dissolving out the alkali metal compounds from the carbon.

4. The process of producing decolorizing 95 carbon, comprising, mixing porous mineral coal with an alkali metal sulfur compound component mixture, heating the substances thus mixed at a temperature of at least 600° C., and separating the carbon from the alkali metal compounds.

5. The process of producing decolorizing 100 carbon, comprising, mixing small grained mineral coal with an alkali metal sulfate, heating the mixture at a temperature of at least 600° C., and dissolving out the alkali metal compounds from the carbon.

6. The process of producing decolorizing 105 carbon, comprising, repeatedly mixing porous mineral coal with an alkali metal sulfate, heating the mixture at a temperature of at least 600° C., and dissolving out the alkali metal compounds from the carbon.

7. The process of producing decolorizing 110 carbon, comprising, mixing small grained mineral coal with an alkali metal sulfate, heating the mixture at a temperature of at least 600° C., dissolving out the alkali metal compounds from the carbon, and repeating such steps up to the transformation of all of the mineral coal into decolorizing carbon.

8. The process of producing decolorizing 115 carbon, comprising, mixing porous mineral coal with an alkali metal bisulfate, heating the mixture at a temperature of at least 600° C., and dissolving out the alkali metal compounds from the carbon.

9. The process of producing decolorizing 120 carbon comprising mixing porous mineral coal with an alkali metal sulphur compound reducible to an alkali metal sulphide upon being heated with carbonaceous mat- 130

ter; heating the mixture under non-oxidizing conditions at a temperature of at least 600° C., and subsequently dissolving out the alkali metal compound from the carbon.

10. The process of producing decolorizing carbon comprising mixing porous mineral coal with an alkali metal sulphur compound reducible to an alkali metal sulphide upon being heated with carbonaceous matter;

heating the mixture under non-oxidizing conditions at a temperature between 650-700° C. for from 30 to 60 minutes and subsequently dissolving out the alkali metal compound from the carbon.

In testimony whereof I have signed my name to this specification.

EMIL HENE.